# EUROPEAN PATENT SPECIFICATION

(11) **EP 2 619 362 B1**
(45) Date of publication and mention of the grant of the patent: **16.06.2021**
(21) Application number: 11827087.5
(22) Date of filing: 20.09.2011
(51) Int. Cl.: D03D 1/00, D03D 13/00, F41H 5/04, D03D 15/00, A41D 31/24

(54) **HIGH PERFORMANCE COMPOSITE FABRIC**
HOCHLEISTUNGSVERBUNDSTOFF
TISSU COMPOSITE HAUTE PERFORMANCE

(30) Priority: 20.09.2010 US 384560 P; 15.06.2011 US 201113161322
(43) Date of publication of application: 31.07.2013
(73) Proprietor: TYR Tactical, LLC, Peoria, AZ 85345 (US)
(72) Inventor: BECK, Jason, R., Peoria AZ 85382 (US)
(74) Representative: Lloyd, Robin
(86) International application number: PCT/US2011/001619
(87) International publication number: WO 2012/039757

(56) References cited:
- WO-A2-2004/089143
- US-A- 5 104 727
- US-A- 5 547 536
- US-A1- 2006 135 022
- US-A1- 2010 080 971
- US-B1- 6 219 842
- None

## Description

### TECHNICAL FIELD

The present invention generally relates to durable fabrics suitable for use in various ruggedized garments, gear, and equipment; including tactical equipment and clothing articles such as anti-ballistic vests and the like.

US2010/080971 discloses an apparatus for providing impact, abrasion and sharp implement resistance to a body. The apparatus including an impact layer having a plurality of plates adhered to a layer of penetration resistant fabric and an energy absorptive layer including an energy absorptive material coupled to the impact layer. The apparatus may further include a layer of woven fabric and a layer of multiple plies of a penetration resistant fabric.

WO2004/089143 discloses a textile structure resistant to perforation, specifically for shoe soles, comprising one or more layers of woven fabric or aramidic fibers and one or more layers of woven fabric of high tenacity non-aramidic fibers; the layers are bonded together by means of thermoplastic film and each separate layer of fabric is treated, preferably in the right side, by coating with polyester and/or acrylic resin enriched with powders of hard and abrasive materials, such as ceramic materials preferably micronized and in the form of aluminum silicates.

### DESCRIPTION OF THE EMBODIMENTS

Although specific terms are employed herein, they are used in a generic and descriptive sense only and not for purposes of limitation. Unless otherwise expressly defined herein, such terms are intended to be given their broad ordinary and customary meaning not inconsistent with that applicable in the relevant industry and without restriction to any specific embodiment hereinafter described. As used herein, the article "a" is intended to include one or more items. Where only one item is intended, the term "one", "single", or similar language is used. When used herein to join a list of items, the term "or" denotes at least one of the items, but does not exclude a plurality of items of the list.

For exemplary methods or processes of the invention, the sequence and/or arrangement of steps described herein are illustrative and not restrictive. Accordingly, it should be understood that, although steps of various processes or methods may be described as being in a sequence or temporal arrangement, the steps of any such processes or methods are not limited to being carried out in any particular sequence or arrangement, absent an indication otherwise. Indeed, the steps in such processes or methods generally may be carried out in various different sequences and arrangements while still falling within the scope of the present invention.

Additionally, any references to advantages, benefits, unexpected results, or operability of the present invention are not intended as an affirmation that the invention has been previously reduced to practice or that any testing has been performed. Likewise, unless stated otherwise, use of verbs in the past tense (present perfect or preterit) is not intended to indicate or imply that the invention has been previously reduced to practice or that any testing has been performed.

An aspect of the invention provides a durable, wear resistant composite fabric, consisting of:
an outer layer made of a woven fabric having a weight between 22-110 Tex (200-1000-denier) nylon; and
a backing layer made of woven fabric comprising para-aramid fibers, the para-aramid fibers having a Tex value of between 11 (100 denier) and 132 (1200 denier) and an aerial density between 0.01 to 0.03 g/cm² (3 and 10 ounces per square yard), the backing layer consolidated with the outer layer.

The synthetic outer layer may be for example a high-performance Nylon-6,6 product presently manufactured by Invista, a wholly owned division of Koch Industries Inc., and sold under the trade name Cordura®. Cordura is used in a wide range of products from luggage and backpacks to boots, military apparel (such as tactical blade sheaths and ammunition pouches), and performance apparel. In one particular embodiment the weight of nylon fabric used in the composite material is about 55 Tex (500 denier).

The backing of the composite material may be made of high tenacity para-aramid fibers. Due to their remarkably high tensile strength-to-weight ratio, such fibers have many applications, including for example bicycle tires, racing sails, mooring lines, and body armor. Specific high tenacity para-aramid fibers suitable for the composite material of the present invention include but are not limited to Kevlar®, a para-aramid synthetic fiber manufactured by DuPont™; Twaron, another para-aramid fiber with roughly the same chemical structure, manufactured by Teijin Aramid.

Also described herein are high tenacity polymer fibers, such as terephthaloyl chloride (TCI), an aramid fiber closely related to para-aramids, also manufactured by Teijin Aramid and sold under the name Technora®; and high molecular weight polyethylene (HMWPE) such as commercially known Spectra®. Other suitable materials include polybenzobisoxazole fibers (PBO) sold under the name ZYLON™ by Toyobo Co. Ltd., of Osaka, Japan, and heat resistant aramid fiber products such as Dupont's Nomex® and Protera® fabrics.

Such fibers may have a tensile strength greater than about 2000 MPa (or greater than about **79N/tex** (7 grams per denier)) and an elastic modulus greater than about 60 GPa. Moreover, there have been generations of fibers and fabrics made from these fibers which have evolved over the years beginning with the first generation of ballistic nylon; second generation of Kevlar® 29, Kevlar® 49, Twaron and Spectra®; third generation of Twaron T-2000 Microfilament, Kevlar® 129 and Kevlar® LT fabrics; and fourth generation of Araflex™

In one exemplary embodiment of the backing layer, high performance para-aramid fibers are utilized in the form of a woven fabric, including for example woven fabrics generally used for repelling and trapping hand driven sharp objects such as knives, awls, shanks and the like. Depending upon the particular intended use, an exemplary woven fabric may be constructed from yarn of anywhere between about 11 Tex (100 denier) and 132 Tex (1200 denier), and aerial densities in the range of 0.01 to 0.03 g/cm² (3 to 10 ounces per square yard "OSY"). For example, fabrics constructed of yarns in the 22 to 33 Tex (200 to 300 denier) range, and aerial densities in the 3 to 4 OSY range are generally preferred for items such as pouches, small duffels, backpacks and the like. Alternatively for heavier applications such as large suitcases or equipment bags, larger yarns in the 77 to 132 Tex (700 to 1200 denier) range, and densities in the 7 to 10 OSY range may be preferable.

The woven fabric of the backing layer may be formed of a relatively tight, puncture resistant weave, comprising for example at least 16 fibers per cm (40 fibers per inch) in a first, or warp direction, and at least 16 fibers per cm (40 fibers per inch) in a second, or fill direction. In one particular embodiment the backing layer comprises a weave with between 24 and 28 fibers per cm (between 60 and 72 fibers per inch) in both the warp and fill directions. In addition, the fabric may be formed by tightly weaving multi-filament yarns to obtain a warp yarn "density" or "cover" in excess of 100 percent at the center of the fill yarn, and a fill yarn density or cover in excess of 75 percent as measured between two warp ends. Such tight weaves may comprise in excess of 39 fibers per cm (100 fibers per inch) in the warp and fill directions, and filament crossovers in the range of about 8 million filament crossovers per square cm (50,000,000 (fifty million) filament crossovers per square inch) up to 14 million filament crossovers per square cm (90,000,000 (ninety million) filament crossovers per square inch). An exemplary tightly woven, puncture resistant fabric suitable for a backing layer is disclosed in US Patent no. 5,565,264.

In one particularly embodiment, the backing layer is Dupont™ Kevlar® Correctional™, a tightly woven Kevlar® fabric. Kevlar Correctional is advertized as an extremely tight weave utilizing filaments one fourth the size of comparable materials. Another suitable commercially available material is a woven puncture resistant product sold under the trademark TURTLESKIN by Warwick Mills, Inc., of New Ipswich, N.H. These products are available in various weights, with 22 Tex (200 denier) and 33 Tex (300 denier) sizes particularly preferred for construction of lightweight personal gear such as packs and pouches, and fabric weights in the 55 Tex (500 denier) to 110 Tex (1000 denier) range preferable for larger, heavier articles such as large suitcases and equipment duffels.

The nylon outer material and backing layer are preferably consolidated, or laminated into a unitary composite fabric using any suitable technique such as bonding, stitching, and the like. Suitable bonding methods include for example the use of various types of adhesives, such as air-drying adhesives, chemically setting adhesives, radiation activated adhesives such as UV activated dental adhesives, hot-melt adhesives, and pressure sensitive adhesives. An adhesive may be pre-applied on at least one of the surfaces or materials to be joined, or separately introduced during a lamination process. In one embodiment, two fabrics layers are laminated under heat and pressure using a solid, polymer based thermoplastic adhesive, such as a polyamide, polyester, elastomeric urethane, or polyolefin polymer. One particular suitable product is a dry, nonwoven mat, or web of a polymer-based thermoplastic manufactured by Spunfab Adhesive Fabrics of Cuyahoga Falls, Ohio. Another suitable material is a class of thermoplastic adhesives by 3M sold under the name "Stitchless Bonding Films". The fabric layers and the thermoplastic adhesive may be supplied from respective adjacent spools, and fed through a laminating machine with the thermoplastic web sandwiched between the fabric layers. An exemplary hot melt laminating process is described for example in US Patent number 5,547,536.

As noted above, the two fabrics of the present invention may also be consolidated using various types of Pressure Sensitive Adhesives, also referred to as "PSA"s. PSAs are distinguished from most other types of adhesives in that they bond on contact, rather than through a solidifying process such as evaporation, chemical reaction, or melting. PSAs are usually based on an elastomer compounded with a suitable tackifier (e.g., a rosin ester). Suitable elastomers include those based on natural rubber, Nitriles, Butyl rubber, Acrylics, Styrene block copolymers, vinyl ethers, Ethylenevinyl acetate, and various silicon rubbers. In one exemplary embodiment the PSA comprises an acrylic adhesive such as 3M's family of VHB TM permanent assembly tapes. Another suitable PSA is 3M adhesive# 9485PC, an acrylic sheet approximately 0.127 mm (5 mils) thick, and sold in rolls up to 122cm (48 inches) wide.

The strength of the high performance fiber backing makes the composite material particularly beneficial in high wear areas of garments or equipment. Examples of high wear areas include corners of ammunition pouches, fragmentation pouches, radio communication pouches, and armor pockets in armor plate carriers. In ballistic vests and ballistic armor carriers the combination of materials also increases longevity and strength of the key load carriage points, particularly once the material is sewn through. Seams can be further strengthened by folding the seam over to double or triple thickness prior to stitching. In addition, any tears or de-laminations in the outer layer can be temporarily field repaired by re-attaching the damaged outer fabric to the intact backing using a fast setting adhesive such as Cyanoacrylate (referred to generically as "Superglue") liquid adhesive. Alternatively, if portions of the outer layer are missing or worn away making reattachment impractical, the intact backing can instead simply be left exposed, and if desired, temporarily disguised using a suitably colored paint or ink marker.

For the purposes of describing and defining the present invention it is noted that the use of relative terms, such as "substantially", "generally", "approximately", and the like, are utilized herein to represent an inherent degree of uncertainty that may be attributed to any quantitative comparison, value, measurement, or other representation. These terms are also utilized herein to represent the degree by which a quantitative representation may vary from a stated reference without resulting in a change in the basic function of the subject matter at issue.

Exemplary embodiments of the present invention are described above. No element, act, or instruction used in this description should be construed as important, necessary, critical, or essential to the invention unless explicitly described as such. Although only a few of the exemplary embodiments have been described in detail herein, those skilled in the art will readily appreciate that many modifications are possible in these exemplary embodiments without materially departing from the novel teachings and advantages of this invention. Accordingly, all such modifications are intended to be included within the scope of this invention as defined in the appended claims.

## Claims

1. A durable, wear resistant composite fabric, consisting of:
an outer layer made of a woven fabric having a weight between 22-110 Tex (200-1000-denier) nylon; and
a backing layer made of woven fabric comprising para-aramid fibers, the para-aramid fibers having a Tex value of between 11 (100 denier) and 132 (1200 denier) and an aerial density between 0.01 to 0.03 g/cm² (3 and 10 ounces per square yard), the backing layer consolidated with the outer layer.

2. The composite material of Claim 1, wherein the backing layer is formed of a puncture resistant, relatively tight weave, comprising at least 16 fibers per cm (40 fibers per inch) in a first, warp direction, and at least 16 fibers per cm (40 fibers per inch) in a second, fill direction.

3. The composite material of Claim 2, wherein the puncture resistant backing layer is **characterized by** a warp yarn density in excess of 100 percent, and a fill yarn density in excess of 75 percent.

4. The composite material of Claim 2, wherein the relatively tight weave of the backing layer comprises filament crossovers in the range of about 8 million to 14 million crossovers per cm² (fifty million to ninety million filament crossovers per square inch).

5. The composite material of Claim 1, wherein the backing layer is consolidated with the outer layer through a laminating process using a thermoset adhesive.

6. The composite material of Claim 1, wherein the backing layer is made of 22 Tex (200-denier) para-aramid fibers.

7. The composite material of Claim 1, wherein the fibers may have a tensile strength greater than about 2000 MPa, and an elastic modulus greater than about 60 GPa.

8. The composite material of Claim 1, wherein the fibers have a tensile strength greater than about 79N/tex (7 grams per denier).

9. The composite fabric of Claim 1, wherein the outer layer is made of 55 Tex (500-denier) nylon and the backing layer is made of 22 Tex (200-denier) para-aramid fibers.

10. The composite fabric of Claim 2, wherein the backing layer is consolidated with the outer layer through a laminating process using a thermoset adhesive.

11. The composite fabric of Claim 2, wherein the backing layer comprises between about 24 and 28 fibers per cm (60 and 72 fibers per inch) in both the warp and fill directions.

12. The composite fabric of claim 1, wherein the backing layer is laminated to the outer layer.

13. The composite fabric of Claim 12, wherein the backing layer is laminated to the outer layer using a thermoplastic adhesive.

14. The composite fabric of Claim 13, wherein the backing layer is laminated to the outer layer using a pressure sensitive adhesive.

## Patentansprüche

1. Langlebiges verschleißfestes Verbundgewebe, bestehend aus:
einer äußeren Schicht aus einem gewebten Gewebe mit einem Gewicht von zwischen 22 und 110 Tex (200-1000 Denier) Nylon; und
einer Trägerschicht aus gewebtem Gewebe, das para-Aramidfasern umfasst, wobei die para-Aramidfasern einen Tex-Wert von zwischen 11 (100 Denier) und 132 (1200 Denier) und eine Flächendichte von zwischen 0,01 und 0,03 g/cm² (3 und 10 ounces per square yard) aufweisen, wobei die Trägerschicht mit der äußeren Schicht konsolidiert ist.

2. Verbundmaterial gemäß Anspruch 1, wobei die Trägerschicht aus einem durchstoßfesten, vergleichsweise dichten Gewebe gebildet ist, das wenigstens 16 Fasern pro cm (40 Fasern pro Inch) in einer ersten, Kettrichtung und wenigstens 16 Fasern pro cm (40 Fasern pro Inch) in einer zweiten, Schussrichtung umfasst.

3. Verbundmaterial gemäß Anspruch 2, wobei die durchstoßfeste Trägerschicht durch eine Kettfadendichte von größer als 100 Prozent und eine Schussfadendichte von größer als 75 Prozent gekennzeichnet ist.

4. Verbundmaterial gemäß Anspruch 2, wobei das vergleichsweise dichte Gewebe der Trägerschicht Fadenüberkreuzungen in dem Bereich von etwa 8 Millionen bis 14 Millionen Überkreuzungen pro cm² (fünfzig Millionen bis neunzig Millionen Fadenüberkreuzungen pro Square Inch) umfasst.

5. Verbundmaterial gemäß Anspruch 1, wobei die Trägerschicht durch ein Laminationsverfahren unter Verwendung eines Duroplastklebstoffs mit der äußeren Schicht konsolidiert ist.

6. Verbundmaterial gemäß Anspruch 1, wobei die Trägerschicht aus 22 Tex (200 Denier) para-Aramidfasern gebildet ist.

7. Verbundmaterial gemäß Anspruch 1, wobei die Fasern eine Zugfestigkeit von höher als etwa 2000 MPa und einen Elastizitätsmodul von höher als etwa 60 GPa aufweisen können.

8. Verbundmaterial gemäß Anspruch 1, wobei die Fasern eine Zugfestigkeit von höher als etwa 79 N/Tex (7 Gramm pro Denier) aufweisen.

9. Verbundgewebe gemäß Anspruch 1, wobei die äußere Schicht aus 55 Tex (500 Denier) Nylon gebildet ist und die Trägerschicht aus 22 Tex (200 Denier) para-Aramidfasern gebildet ist.

10. Verbundgewebe gemäß Anspruch 2, wobei die Trägerschicht durch ein Laminationsverfahren unter Verwendung eines Duroplastklebstoffs mit der äußeren Schicht konsolidiert ist.

11. Verbundgewebe gemäß Anspruch 2, wobei die Trägerschicht sowohl in der Kett- als auch in der Schussrichtung zwischen etwa 24 und 28 Fasern pro cm (60 und 72 Fasern pro Inch) umfasst.

12. Verbundgewebe gemäß Anspruch 1, wobei die Trägerschicht an die äußere Schicht laminiert ist.

13. Verbundgewebe gemäß Anspruch 12, wobei die Trägerschicht unter Verwendung eines Duroplastklebstoffs an die äußere laminiert ist.

14. Verbundgewebe gemäß Anspruch 13, wobei die Trägerschicht unter Verwendung eines Haftklebstoffs an die äußere Schicht laminiert ist.

## Revendications

1. Toile composite durable, résistante à l'usure, constituée par :
une couche externe faite dans un tissu de nylon ayant un poids compris entre 22 et 110 tex (200-1000 deniers) ; et
une couche de doublure faite dans un tissu comprenant des fibres de para-aramide, les fibres de para-aramide ayant une valeur en tex comprise entre 11 (100 deniers) et 132 (1200 deniers) et une masse surfacique comprise entre 0,01 et 0,03 g/cm² (3 et 10 onces par yard carré), la couche de doublure étant consolidée avec la couche externe.

2. Matériau composite de la revendication 1, dans lequel la couche de doublure est constituée d'une armature résistante à la perforation, relativement serrée, comprenant au moins 16 fibres par cm (40 fibres par pouce) dans une première direction, de chaîne, et au moins 16 fibres par cm (40 fibres par pouce) dans une deuxième direction, de trame.

3. Matériau composite de la revendication 2, dans lequel la couche de doublure résistante à la perforation est **caractérisée par** une densité de fils de chaîne dépassant 100 pour cent, et une densité de fils de trame dépassant 75 pour cent.

4. Matériau composite de la revendication 2, dans lequel l'armature relativement serrée de la couche de doublure comprend des croisements de filaments dans la gamme d'environ 8 millions à 14 millions de croisements par cm² (cinquante millions à quatre-vingt-dix millions de croisements de filaments par pouce carré).

5. Matériau composite de la revendication 1, dans lequel la couche de doublure est consolidée avec la couche externe par un procédé de contrecollage utilisant un adhésif thermodurcissable.

6. Matériau composite de la revendication 1, dans lequel la couche de doublure est constituée de fibres de para-aramide de 22 tex (200 deniers).

7. Matériau composite de la revendication 1, dans lequel les fibres peuvent avoir une résistance à la traction supérieure à environ 2000 MPa, et un module d'élasticité supérieur à environ 60 GPa.

8. Matériau composite de la revendication 1, dans lequel les fibres ont une résistance à la traction supérieure à environ 79 N/tex (7 grammes par denier).

9. Toile composite de la revendication 1, dans laquelle la couche externe est constituée de nylon de 55 tex (500 deniers) et la couche de doublure est constituée de fibres de para-aramide de 22 tex (200 deniers).

10. Toile composite de la revendication 2, dans laquelle la couche de doublure est consolidée avec la couche externe par un procédé de contrecollage utilisant un adhésif thermodurcissable.

11. Toile composite de la revendication 2, dans laquelle la couche de doublure comprend entre environ 24 et 28 fibres par cm (60 et 72 fibres par pouce) dans les directions à la fois de chaîne et de trame.

12. Toile composite de la revendication 1, dans laquelle la couche de doublure est contrecollée à la couche externe.

13. Toile composite de la revendication 12, dans laquelle la couche de doublure est contrecollée à la couche externe au moyen d'un adhésif thermoplastique.

14. Toile composite de la revendication 13, dans laquelle la couche de doublure est contrecollée à la couche externe au moyen d'un adhésif sensible à la pression.
